

Sept. 19, 1939.

G. WASSERMANN  
METHOD FOR MANUFACTURING MAGNETIC MATERIAL  
OF HIGH PERMEABILITY IN SHEET FORM  
Filed March 6, 1937

2,173,240

Fig. 1



Fig. 3



inventor:

Günther Wassermann

by *Albright Bros.*  
his attorney

## UNITED STATES PATENT OFFICE

2,173,240

METHOD FOR MANUFACTURING MAGNETIC  
MATERIAL OF HIGH PERMEABILITY IN  
SHEET FORM

Günter Wassermann, Berlin-Wilmersdorf, Germany, assignor to Siemens &amp; Halske, Aktiengesellschaft, Siemensstadt, near Berlin, Germany, a corporation of Germany

Application March 6, 1937, Serial No. 129,362  
In Germany March 6, 1936

## 3 Claims. (Cl. 148—12)

My invention relates to a method for manufacturing magnetic material of high permeability in sheet form. It is illustrated in the accompanying drawing, in which

5 Fig. 1 represents a diagrammatic illustration of crystal position.

Fig. 2 diagrammatically represents test results, and

10 Fig. 3 diagrammatically represents an arrangement for transverse rolling.

The structure of the material resulting from the rolling of metals with body centered atom lattices is simple as compared to the face centered metals. As will be seen from the position *a* in Fig. 1 the crystals lie in a position in which the diagonal *d* of one of the surfaces of a cube is located in parallel relation to the direction of rolling and this cube surface is in the ideal case parallel to the plane of the rolled sheet iron. However, this ideal position can- 20

not be practically attained for all crystals. The accompanying dispersion (which is always present also in the best structures) consists in a deviation which is produced by rotation of the 25 crystals approximately  $\pm 40^\circ$  about the face diagonal *d* lying in the direction of rolling. Positions *b* and *c* show schematically two such positions of dispersion. The position for the direction of the easiest magnetization—namely, 30

the direction along the edge of the cube, which in the illustrated ideal position *a* is located in the plane of the sheet iron at an angle of  $45^\circ$  to the direction of rolling and to the transverse direction, that is to say, is quite favorable for 35

magnetic purposes—is changed and the cube is rotated by the dispersion out of the plane of the sheet iron into positions whose geometric locus is a cone about the direction of rolling with an opening angle of approximately  $45^\circ$ . 40

The conditions for a magnetically favorable behavior of this structure are only fulfilled if it is possible to reduce the dispersion so that the edges and the planes of the cube lie to a great extent only in the plane of the sheet iron. A 45 known process shows a method for solving this problem which consists in rolling the sheet iron a number of times alternately in two directions at right angles to one another and to thereby very gradually roll the material down to the desired thickness. In Fig. 1, for instance, one of these two directions (longitudinal rolling) is indicated by an arrow marked LR, and the other direction (transversal rolling) by an arrow marked TR. The cross-rolling operation leads 50

55 to a structure in which the crystals in a pre-

pondering number are located in the ideal position, for the positions of dispersion characteristic of one rolling direction are not suitable for the structure characteristic of the other direction and vice versa, and these crystal positions are, therefore, always destroyed during the next 5 rolling operation.

The manufacture of materials in sheet form and particularly in bands or tapes by the repeated cross-rolling process as heretofore practiced presents, however, certain technical difficulties. In the normal longitudinal rolling process, the material retains its width quite well so that also the length of the rolls may remain the same during the rolling process. However, 10 when cross-rolling the material, the length and the width of the sheet increase to the same extent. The material must, therefore, be often cut, which may be avoided for thin sheet iron to a certain extent only by the use of very long rolls. 15

This disadvantage is removed by the method according to the invention which requires only one change of the direction of rolling. The method consists in first cold rolling the ferromagnetic specimen down to about one-eighth to 20 one-tenth of its original thickness and in subsequently cold rolling it in a direction which is displaced  $90^\circ$  with respect to the first direction of rolling, down to about half the thickness attained after the first rolling operation, which 25 thickness is the final, desired one.

The tests carried out in this connection had the following result which is diagrammatically represented in Fig. 2. In this figure the percentage of reduction in thickness by the first rolling process is plotted against the percentage of reduction in thickness by the second rolling process in a direction at right angles to the direction of the first process. The rolling ratios represented by the encircled points showed in the 30 tests that the crystal orientation produced by the first rolling direction was preponderant, the ratios represented by the heavy solid points showed the orientation of the second rolling direction to be preponderant, and the ratios represented by the crossed points showed that the orientation effects of both rolling directions were 35 equal. For further elucidating the way of registering used in the diagram, an example may be 40 taken in view. Point A in Fig. 2 represents a sheet iron treated as follows. The sheet was first cold rolled with a rolling degree of 82% (see abscissa), that is, reduced to a thickness of a little more than  $\frac{1}{5}$  of the original thickness. Then a crosswise rolling was applied resulting 45

5

10

15

20

25

30

35

40

45

50

55

in a further reduction of 50% (see ordinate). The fact that dot A is of heavy solid type also shows that after these treatments the effect of the second rolling was preponderant as manifested by a crystal orientation corresponding to the direction of the second cold rolling operation.

The range of percentage of reduction employed in the first cold rolling operation was selected between 82-95% with a sheet iron thickness between 1.2 and 0.3 mm. after the first rolling. It is not convenient to employ sheet iron with a lower degree of reduction for the first rolling operation, since the structure in this material is still far from being properly developed. The tests showed that during the second rolling operation, in a direction 90° displaced from the first rolling direction, the dispersion decreases about the first direction of rolling. The structure becomes symmetrical with respect to both directions and, on further rolling in the second direction, finally the dispersion increases considerably about the second direction of rolling, so that a normal structure of the rolled material 25 is again attained.

When employing reductions below 36% for the second direction of rolling the points 1, 1, 1 show that the orientation resulting from the first rolling was always predominant. In the case of 30 sheet iron prerolled to a reduction by 90 to 95%, a symmetrical structure was attained when the material obtained from the rolling in the first direction was reduced by 50-55% in the second direction (points 2, 2, 2), and in the case of sheet iron prerolled to a reduction by 82% symmetry 35 was attained already by reducing it 40% during rolling in the second direction. With higher degrees of reduction in the second direction, the structure resulting from this direction of rolling is in most cases predominant.

40 This result means that a material rolled in sheet form in one direction, for instance from 6 mm. to 0.6 mm. need only be additionally rolled to 0.3 mm. transversely to the first direction of rolling and to its final gauge in order to attain a symmetrical structure. Consequently, in the 45 first direction of rolling, the material must be lengthened to about ten times its original length, whereas in the second direction of rolling only to two times the length, and thus the cross-rolling 50 process is considerably simplified.

The method according to the invention may 55 also be applied to the manufacture of steel tape for armoring purposes or the like. The first rolling operation is effected in this case in the normal manner heretofore practiced. For the second rolling operation, rolling mills as shown in Fig. 3 are employed which permit a lateral passage of the tape through the housings in which the 60 bearings of the top and bottom rolls are spaced from one another. The tape is fed in parallel relation to the axes of the rolls and cross-rolled. After one or more passages through the rolls the tape is advanced an amount equal to the length 65 of the roll and is then again cross-rolled etc.

To attain a high permeability and low losses the material with body centered crystal grids must be annealed after the rolling operation. However, during this annealing treatment, the uniform structure attained by the rolling operation should be largely maintained. In order that the crystals formed during the recrystallization have as far as possible the orientation of the deformed crystals it is necessary that the annealing treatment be carried out at low temperatures.

10 Tests carried out in this connection have shown that these conditions are fulfilled to the greatest possible extent, if the annealing treatment is effected at temperatures lying between 600 and 1,000 degrees centigrade. Annealing temperatures of 800 to 900 degrees centigrade proved particularly favorable, since after such a heat treatment the structure has, on the one hand, still a good appearance and the sheet iron is capable of being easily deformed and, on the other hand, 15 comparatively high values of permeability may be attained.

I claim as my invention:

1. A method of manufacturing magnetic materials of high permeability in sheet form from 25 materials with body-centered cubic atom lattices consisting in first cold rolling the specimen to reduce it to about one-eighth to one-tenth of its original thickness, in subsequently cold rolling it in a direction displaced 90° with respect to the 30 first rolling direction to reduce it to about half the thickness attained after the first rolling, and representing the final thickness, and in then heat treating the specimen at temperatures lying between 600 and 1000 degrees centigrade.

35 2. A method of manufacturing magnetic materials of high permeability in tape form from materials with body-centered cubic atom lattices consisting in longitudinally cold-rolling the material to reduce it to one-eighth to one-tenth 40 of its original thickness, in subsequently rolling it in a direction displaced 90° with respect to the first direction of rolling to reduce it to approximately one-half of the thickness attained by the longitudinal rolling and in a rolling mill through 45 which the tape is fed in parallel relation to the axes of the rolls and cross-rolled in several passes to the aforesaid thickness as the final form, and in subsequently heat treating the finally rolled tape at temperatures lying between 600 and 1000 50 degrees centigrade.

3. A method of manufacturing magnetic materials of high permeability in sheet form from iron-silicon alloys containing up to 5% silicon 55 consisting in cold rolling the material to reduce it to one-eighth to one-tenth of its original thickness, in subsequently rolling it in a direction displaced 90° with respect to the first direction of rolling to reduce it to approximately one-half of the thickness attained by the first rolling, and 60 representing the final thickness, and in subsequently heat treating the finally rolled material at temperatures lying between 300 and 900 degrees centigrade.

GÜNTER WASSERMANN. 65